

A. J. HAIN.  
PROCESS OF PREPARING PRINTING PLATES.  
APPLICATION FILED JUNE 11, 1917.  
**1,346,885.**

Patented July 20, 1920.



*INVENTOR.*  
Albert J. Hain  
By Brockett and Hyde  
Atty's.

# UNITED STATES PATENT OFFICE.

ALBERT J. HAIN, OF LAKEWOOD, OHIO.

## PROCESS OF PREPARING PRINTING-PLATES.

1,346,885.

Specification of Letters Patent.

Patented July 20, 1920.

Application filed June 11, 1917. Serial No. 174,049.

*To all whom it may concern:*

Be it known that I, ALBERT J. HAIN, citizen of the United States, residing at Lakewood, in the county of Cuyahoga and State 5 of Ohio, have invented certain new and useful Improvements in Processes of Preparing Printing-Plates, of which the following is a specification.

This invention relates to a process of preparing printing plates, and more especially 10 printing plates of the half tone variety such as are used in newspaper, magazine and like work for printing reproductions of photos, cuts and the like.

15 The object of the invention is to provide an improved process which is simple and does away with considerable of the apparatus, such as cameras, screens and the like usually employed in process work, thereby enabling 20 the proper effects to be obtained with less apparatus and requiring a minimum amount of skill, and adapting the process to be performed, for example, in small printing plants or by amateurs without employment 25 of the apparatus customarily found in fully equipped plants for this purpose.

Further objects of the invention are in 30 part obvious and in part will appear more in detail hereinafter.

35 The invention comprises the several process steps hereinafter described and claimed.

In the drawings Figure 1 represents a 40 diagrammatic cross sectional view, enlarged, illustrating the preparation of a plate for printing by one specific process embodying the invention; Fig. 2 is a plan view, illustrating the treatment of and effect upon the 45 isolated protecting areas; and Figs. 3 and 4 are diagrammatic sectional views, enlarged, 50 illustrating other specific ways of carrying out the invention.

It will of course, be understood that the 55 result to be accomplished is the production of a printing plate whose surface has been interrupted, by etching or the like, as is usual, to leave upon it unaffected areas which will print out in black upon the paper, with intervening areas which have been hollowed out and therefore will not print, or vice 60 versa, in intaglio engraving. The extent or value of the unaffected areas in any region, of course, varies with the lights and shadows of the image to be printed, and will be of greater area or higher value where the picture 65 is shaded or darker than at the higher lights. This plate is usually formed by

etching a smooth surfaced metal plate, such as a zinc plate, the etching effect being limited to certain areas by the formation upon the plate of a resist which prevents the etching fluid from attacking the plate at the areas to be unaffected. The particular purpose of the present invention is to provide an improved method or process of building up upon the plate in skeleton form the 60 proper resist to confine the action of the etching fluid to certain desired areas and prohibit its action upon other areas.

Briefly stated, therefore, the invention consists in first forming upon the plate to be 65 etched a series of closely and uniformly spaced protecting areas, all of uniform size, adapted in one way or another to protect the plate from the action of the etching fluid, and subsequently treating said spaced protecting 70 areas, to vary their size in accordance with variations in the lights and shadows of the image, as a consequence of which the plate finally produced, when used as a printing 75 plate, will reproduce the light and shadow effects of the image.

The invention, therefore, proceeds from an initial step of first forming this series of uniformly spaced protecting areas of uniform size. Said areas should preferably be 80 of what may be termed minimum size, as they are usually not reduced in size by a subsequent step and will therefore produce their counterpart dots or stippling even in the highest lights of the image, except as their size 85 effect may be diminished by undercutting action of the etching fluid. The protecting areas are also isolated from each other. In other words, they do not merge into each 90 other, at least so far as their protecting effect 95 upon the plate is concerned, thereby enabling them to be built up or enlarged radially in all directions. Nevertheless, they may be part and parcel of the same layer, film or stratum, different portions of which are affected in 100 different ways to form isolated protecting areas on the one hand, and intervening areas which do not have a protecting effect, on the other hand.

The isolated protecting areas may be 105 formed directly upon the surface of the plate to be etched and themselves have the quality of preventing action on the plate by the etching fluid. On the other hand, it is sometimes more convenient to first cover the plate 110 with a layer of a resist which will protect the plate from acid, and upon said resist

applying isolated protecting areas of a material which will serve as a resist to a reagent for attacking the substratum or initial resist layer. In this case the isolated protecting areas are formed and built up according to the lights and shadows of the image, then used to protect areas of the substratum while attacking the intervening areas, thereby exposing or opening up through the substratum the metal of the base plate to attack by the etching fluid, or even to permit attack of the base plate through the unaffected intervening areas without disturbing them.

The character of resists and reagents used is immaterial so long as the foregoing effects are obtained by the means and in the manner specified, but to more completely set forth the invention, and purely for the purposes of illustration, I will now describe several methods employing the invention.

According to the first method the plate to be etched, which may be of zinc or some other well known material for this purpose and which is indicated at 1, is first covered with a layer 2 of a material resistant to the particular etching fluid to be used, such as an acid resist. This acid resist may be of any suitable material several of which are well known, for example, gum dammar, gum shellac, bitumen, dragon's blood, or copper plate. In the present instance, however, we will assume that the resist is copper plate upon the surface of the zinc.

Over the copper resist is applied a film 3 of a colloid or emulsion, such as gelatin or the like. After this film has been treated the plate is immersed in a suitable sensitizing solution, preferably one containing salts of manganese. One solution suitable for the purpose is as follows:

*Solution A.*

|                                          |    |         |
|------------------------------------------|----|---------|
| Saturated solution potassium bi-chromate | 5  | drams.  |
| 45 Manganous sulfate                     | 44 | grains. |
| Manganous chlorid                        | 22 | grains. |
| Aluminum sulfate                         | 10 | grains. |
| Water to make                            | 1½ | ounces. |

50 The sensitized colloid plate is then dried and is exposed to the action of light beneath a high-light photo engraver's screen having regularly spaced openings or transparent areas. The effect of such exposure is to produce a hardening effect upon the sensitized colloid where the light penetrates the photo engraver's screen, but without effect upon the colloid where the light does not penetrate the screen, thereby producing upon the 55 sensitized plate the counter part of the photo engraver's screen as a series of uniformly spaced isolated areas 4, shown considerably enlarged in Fig. 1, of minimum uniform size and of hardened colloid material, in a continuous layer with intervening areas 5 of un-

affected unhardened colloid material. At the same time exposure to light produces a chemical effect upon the reagents in the sensitized film so that the isolated areas 4 of the hardened colloid are impregnated with an 70 insoluble manganous oxid. The exposed plate is then washed for three minutes, more or less, in cold water, or until all the soluble unaffected bichromate and manganous salts are washed out. The cold water does not 75 affect the colloid itself.

The plate, produced as above described, is used in connection with a print in metallic silver, such for instance as a print which has been obtained, in the well known manner, 80 with a silver bromid emulsion. Such a print is immersed in a suitable reducing solution, for example as follows:—

*Solution B.*

|                  |    |         |
|------------------|----|---------|
| Copper sulfate   | 96 | grains. |
| Potassium bromid | 48 | grains. |
| Water            | 2  | ounces. |

When the image is fully bleached the print is well washed with water and is immersed 90 for a minute in a solution as follows:

*Solution C.*

|               |     |         |
|---------------|-----|---------|
| Sulfuric acid | 1   | dram.   |
| Alum          | 120 | grains. |
| Water         | 20  | ounces. |

The print, thus prepared, and indicated at 6, is then brought into close contact with the treated colloid surface of the plate to be 100 etched, the contact being maintained for some time, say about twenty minutes, after which the print is removed.

The effect of the contact treatment is to cause the manganous oxid in the isolated 105 protecting areas of the colloid film to oxidize and render insoluble the surrounding tissues of the colloid film, as at 7, in proportion to the amount of silver in the original print to be reproduced. In other words, where, 110 in the original print a maximum amount of silver existed, as at a deep shadow, the maximum amount of hardening action has extended into the tissues of the colloid surrounding the several isolated protecting areas in that neighborhood of the print being formed; where there was little or no silver in the original print, as at a high light, there is little or no hardening action in the print being formed and the isolated areas in 115 that neighborhood are unaffected.

The plate is next dried, alcohol being used to assist the action, if desired, and is immersed in a solution of ferric chlorid 42° Baumé, which quickly penetrates the colloid where it has not been hardened or rendered insoluble, and removes the acid resisting copper substratum. The plate is then ready for etching with a suitable acid, such as nitric acid diluted in water.

If an acid resisting substratum, such for example as a solution of asphalt in benzol or shellac in alcohol has been used in place of copper, then after removing the print from contact with the plate the soluble colloid may be washed out with hot water, thus exposing the acid resisting substratum, which is removed, where unprotected, by a suitable solvent, such as alcohol for shellac or turpentine for asphalt, whereupon the plate is etched with acid as before.

Up to this point I have described the formation of what may be termed a built up skeleton of the image upon a resisting substratum, and the removal of the unprotected areas of the substratum to expose the base plate for etching. The same kind of a built up skeleton image in gelatin may be formed directly on the surface to be etched, which may be zinc, copper or the like, and then said skeleton image may be burned into the metal plate to convert it into a protecting enamel, so that the burned skeleton image itself becomes a resist for the etching fluid. This does away with the additional resisting substratum and the built up protecting areas themselves become the resist, as before stated.

In the first method described the uniform isolated protecting areas of minimum size are built up or increased in size in varying amounts according to the lights and shadows of the image by the effect of the silver in the bromid print upon the manganous oxid in the isolated areas, and the hardening action of the two upon the neighboring colloid tissues, but it is not essential that the silver for producing this action be in a print brought into contact or juxtaposition with the colloid of the plate. The silver may be embodied in various ways in the plate itself, thereby rendering the plate suitable for direct exposure to the action of light under a negative or in a camera. A method of this kind, for example, would be practised as follows:

Upon the plate to be etched, indicated at 10, Fig. 3, is placed a suitable acid resisting substratum or layer 11. The resist for this specific illustration may be assumed to be compounded as follows:

#### Resist X.

|                 |            |
|-----------------|------------|
| Syrian asphalt  | 1 ounce.   |
| 55 Benzol       | 15 ounces. |
| Oil of lavender | 1 dram.    |
| Turpentine      | 1 dram.    |

Upon the resist are formed a series of closely and uniformly spaced isolated protecting areas of uniform minimum size, indicated at 12, in which may be incorporated manganous oxid by the use of a solution, such as Solution A, above. For example these isolated areas may be formed upon the

plate by flowing over it and drying thereon an even film of a colloid compounded as follows:

#### Colloid M.

|         |            |
|---------|------------|
| Gelatin | 70 grains. |
| Water   | 1 ounce.   |

This colloid film when dried is sensitized by immersion three minutes in Soluton A, and, when dried, is exposed beneath a high-light photo engraver's screen until the light has rendered insoluble those uniformly spaced minimum sized areas exposed to the light. The soluble portion of the film is then washed out in warm water, leaving upon the plate the isolated protecting areas 12, insoluble and impregnated with manganous oxid:

The plate is then flowed with an emulsion or colloid film 13 of sensitive form, preferably containing a silver salt, such as silver bromid. One suitable sensitized film for this purpose is compounded as follows:

|                                                          |            |
|----------------------------------------------------------|------------|
| Gelatin                                                  | 80 grains. |
| Ammonium bromid                                          | 30 grains. |
| Water                                                    | 1 ounce.   |
| Silver nitrate, 30 grains dissolved in 1 ounce of water. |            |

When the sensitized film is dried, the prepared plate is used by exposing it beneath a photographic negative, or, for some purposes, in a camera. It is then developed in any suitable developing agent and is fixed in a mixture of sodium thiosulfate ("hypo"), after which the plate is immersed in a solution as follows:

#### Solution D.

|                       |            |
|-----------------------|------------|
| Potassium ferricyanid | 5 grains.  |
| Potassium bromid      | 20 grains. |
| Water                 | 1 ounce.   |

The purpose and effect of this solution are to render the gelatin emulsion or colloid insoluble or hard in the presence of silver bromid where in contact with the oxidized isolated protecting areas surrounded by said colloid film, as at 14, the effect being in proportion to the exposure of each area and the deposit of silver bromid remaining in the sensitized film in the neighborhood of such area. After this treatment the soluble film in the intervening spaces 15 between the isolated areas is washed out with warm water. The acid resisting substratum, where unprotected by the remaining gelatin is dissolved in a suitable solvent, such as turpentine, and the plate is etched with a suitable etching medium, such as a solution of nitric acid in water in case the base material of the plate is zinc.

In this last method the silver deposit is created in the body of the sensitized colloid film superposed upon previously formed iso-

lated protecting areas, said isolated areas being then built up by reason of the juxtaposition of the silver deposits in the tissues neighboring each isolated area when the 5 plate is treated with the reducing solution, such as Solution D. The silver deposit, however, may be incorporated directly into the bodies of the isolated areas, doing away therefore with the necessity of preparing 10 and flowing upon the plate a sensitized film, and enabling a plain colloid film to be utilized, if desired. One method embodying this form of the invention is practised as follows:

15 Upon the plate to be etched, indicated at 20, Fig. 4, is placed a layer 21 of a suitable resist, such as Resist X before mentioned. Upon this resist are formed the isolated protecting areas, in which may be incorporated 20 a light sensitive element. This may be accomplished as follows:—

A colloid film, such as the colloid or emulsion M before referred to, is flowed over the plate and dried, after which it is sensitized 25 by immersion three minutes in the following solution:—

*Solution E.*

Potassium bichromate 10 grains.  
30 Water 1 ounce.

The plate when dry is exposed beneath a high light photo engraver's screen to harden the exposed areas 22, the soluble portions of the film being then washed out in water.

35 The plate is then immersed in a solution as follows:—

*Solution F.*

Potassium bromid 30 grains.  
40 Acetic acid 1 drop.  
Water 1 ounce.

The plate is then dried and immersed in a solution as follows:

*Solution G.*

Silver nitrate 30 grains.  
Citric acid 5 grains.  
Distilled water 1 ounce.

50 This treatment directly sensitizes with silver bromid the isolated protecting areas 22, which are formed of a colloid film. The protecting areas are then furnished with a surrounding body from whose tissues they 55 may be subsequently built up in accordance with the lights and shadows of the image, for which purpose the plate is flowed with a simple emulsion or colloid film 23, composed, for example, as follows:—

60 Gelatin 70 grains.  
Water 1 ounce.

The plate, thus treated, is exposed beneath a photographic negative, or, for some pur-

poses, in a camera, and is developed and 65 fixed as usual.

The plate is then treated by any suitable method to obtain the image in halftone dot form upon the acid resisting substratum. Two such methods may be described for purposes of illustration. The first method is as follows:—

**FIRST METHOD.**

The plate is flowed with a solution as follows:—

*Solution H.*

|                                  |           |
|----------------------------------|-----------|
| Pyrogallic acid                  | 3 grains. |
| Citric acid                      | 3 grains. |
| Water                            | 2 ounces. |
| 20-grain silver nitrate solution | 15 drops. |

This solution serves as an intensifier, increasing the deposit of metallic silver upon the exposed isolated protecting areas in accordance with the amount of silver already present in such areas. In other words, in an area containing no silver there is no further or additional deposit, but in all areas containing silver the additional silver deposit is in proportion to the amount already present. The plate is then immersed in a 10% solution of potassium bichromate, which hardens the gelatin in the presence of the metallic silver, and at the same time builds up and increases the size of the isolated protecting areas in accordance with the amount of silver deposit thereon, and therefore in accordance with the lights and shadows of the image. The soluble gelatin is then washed out with warm water, the acid resisting substratum is dissolved with turpentine and the plate is etched as before.

**SECOND METHOD.**

The plate, prepared with the light sensitive isolated areas thereon, may be immersed in a solution as follows:—

*Solution I.*

|                       |            |
|-----------------------|------------|
| Potassium bromid      | 20 grains. |
| Potassium ferricyanid | 5 grains.  |
| Potassium bichromate  | 10 grains. |
| Water                 | 1 ounce.   |

The purpose and effect of this solution are to produce a chemical reaction between the metallic silver deposited in the light sensitive isolated areas and the solution, which makes insoluble the tissues of the plain colloid film neighboring such areas and in direct proportion to the amount of silver contained in such areas. The soluble gelatin is then washed out in warm water, the acid resisting substratum is dissolved and the plate is etched, as before.

While in the specification I have described a number of specific methods employed in the practice of the invention, it

is of course to be understood that the method is capable of considerable modification, within the scope of the appended claims, without departing from the spirit of the invention, and is therefore not limited to the specific methods described. The invention can be carried out with simple apparatus and therefore enables plates of this kind to be prepared by amateurs or in small 10 printing shops without a complete photo engraver's plant, such as is usually necessary.

As to all subject matter common to the two applications, the present application is 15 a continuation of my prior application for process for producing printing plates, filed October 22, 1915, Serial No. 57,247, but the invention of the present application, in certain respects is also an improvement upon 20 that of my prior application, as will be readily understood.

What I claim is:—

1. The method of preparing plates for printing reproductions of an image, consisting in forming upon a plate uniform isolated protecting areas of minimum size, and increasing the size of said areas in every region of the plate in accordance with the value of the light or shadow in that region 30 of the image to be reproduced.

2. The method of preparing plates for printing reproductions of an image, consisting in forming upon a plate uniform isolated protecting areas of minimum size sur-

rounded by neighboring material, and increasing the size of said isolated areas by accretion from said material in every region of the plate in accordance with the value of the light or shadow in that region of the image to be reproduced. 35

3. The method of preparing plates for printing reproductions of an image consisting in forming upon a plate uniform isolated protecting areas of minimum size surrounded by neighboring tissues, increasing 40 45 the size of said isolated areas by accretion from said tissues in every region of the plate in accordance with the value of the light or shadow in that region of the image to be reproduced, and treating the remaining intervening non-projecting areas to expose the 50 plate to the action of an etching fluid.

4. The method of preparing plates for printing reproductions of an image, consisting in depositing upon a plate a uniform 55 continuous layer of a material resistant to an etching fluid, superposing upon said layer a series of uniform isolated protecting areas of minimum size, increasing the size of said areas in every region of the plate in accordance with the value of the light or shadow in that region of the image to be reproduced, and dissolving the layer of resist where exposed between the built up isolated 60 65 protecting areas.

In testimony whereof I affix my signature.

ALBERT J. HAIN.